

No. 811,143.

PATENTED JAN. 30, 1906.

H. HARMET.

COMPRESSING STEEL IN CONICAL MOLDS.

APPLICATION FILED OCT. 7, 1902.

3 SHEETS—SHEET 1.

Fig. 1.



Witnesses  
Thomas M. Smith.

Jas. C. Wobensmith

Inventor  
Hans Harmet,  
By J. Walter Douglas,  
Attorney.

No. 811,143.

PATENTED JAN. 30, 1906.

H. HARMET.

COMPRESSING STEEL IN CONICAL MOLDS.

APPLICATION FILED OCT. 7, 1902.

3 SHEETS—SHEET 2.

Fig. 2.



Witnesses:

Henry E. Everding.  
Jas. C. Wobensmith.

Inventor:

Henry Harmet,  
and J. Walter Douglas  
attorney.

No. 811,143.

PATENTED JAN. 30, 1906.

H. HARMET.

COMPRESSING STEEL IN CONICAL MOLDS.

APPLICATION FILED OCT. 7, 1902.

3 SHEETS—SHEET 3.

Fig. 3.



Witnesses:

Wilhelm Togt  
Thomas M. Smith

Inventor:  
Henri Harmet  
by J. Walter Douglass  
Attorney.

# UNITED STATES PATENT OFFICE.

HENRI HARMET, OF ST. ETIENNE, FRANCE.

## COMPRESSING STEEL IN CONICAL MOLDS.

No. 811,143.

Specification of Letters Patent.

Patented Jan. 30, 1906.

Application filed October 7, 1902. Serial No. 126,294.

*To all whom it may concern:*

Be it known that I, HENRI HARMET, engineer, a citizen of the Republic of France, residing at St. Etienne, Loire, France, have invented certain new and useful Improvements in Compressing Steel in Conical Molds, of which the following is a specification.

The compression of steel as described in my former patent, No. 679,072, dated July 23, A. 10 D. 1901, in conical molds consists in causing the ingot to advance during solidification in a conical ingot-mold by pushing it from the larger end toward the smaller end. To obtain a good compression, the advance of the 15 metal from the base of the conical mold should be such that the resulting reduction in the volume of the ingot is equal to or even greater than the contraction of the metal during the same time. In applying this 20 known process of mine of compressing the ingot any mechanical means may be adopted by which the ingot can be caused to advance in the conical ingot-mold by pushing its larger end toward the smaller end of the cone, 25 the advance being such that the reduction of volume of the ingot is at least equal to the contraction of the metal. The ingot-mold may be in any position provided that the advance of the ingot in the cone can be obtained 30 as desired. Any force also may be employed for producing the advance, such as hydraulic or any other power. In the specification of my former patent, No. 679,072, dated July 23, 1901, and of my application, Serial No. 35 99,335, filed March 21, 1902, I have described the two most important mechanical arrangements for obtaining the advance to the desired extent when the axis of the cone of the ingot-mold is vertical, the larger section being 40 at the bottom and the smaller section at the top. Generally the advance of the ingot in the cone is obtained by keeping the ingot-mold approximately stationary and raising by the press the movable bottom to push the 45 metal in front of it.

In the arrangement I prefer to employ in carrying out the present invention the axis of the cone is vertical and the larger section is at the top. I have shown this preferred 50 arrangement in the annexed drawings, in which—

Figure 1 is the general sectional elevation of an apparatus embodying main features of my invention. Fig. 2 is a vertical section, on a

larger scale, of the ingot-mold; and Fig. 3 is a 55 sectional elevation of a modified form of the apparatus.

The arrangement of the larger section at the top and the smaller one at the bottom is convenient in certain cases—for very small 60 ingots, for example—the casting being so performed that the liquid metal or the ingot is carried by its smaller end, which serves as a base and rests on a movable bottom sufficiently supported to sustain the metal, but 65 which descends vertically when a heavy pressure is placed on the larger end of the ingot. The compression is then effected by submitting the larger end of the ingot to a pressure sufficient to force it into the cone in a manner 70 similar to that adopted when the larger end is at the bottom and the smaller end is at the top, the principle of operation remaining the same. Whatever may be the arrangement adopted, the operation is according to this invention continued until the ingot is completely forced out of the smaller end of the 75 conical ingot-mold, and preferably this is done with the larger end of the mold at the top and in two operations, as follows: The 80 metal having been poured into the ingot-mold  $\alpha$ , the larger end being at the top and the smaller end resting on a base  $m$ , which can descend under a heavy pressure, the larger end of the ingot  $c$  is exposed, by means 85 of the ram  $n$  of the press A, Fig. 1, to the pressure necessary to cause it to advance in the mold  $\alpha$  and to produce a reduction in its volume corresponding to the contraction which takes place during the same time. Af- 90 ter the first period, the metal having approxi- 95 mately solidified, the ingot-mold  $\alpha$ , with the ingot  $c$  in it, is taken to another press B, having a ram  $o$  smaller than the small end of the cone of the ingot-mold, and the ingot, which has already solidified, is then further made to advance in the cone until it is forced out at the smaller end, which is left open, the ingot-mold  $\alpha$  during this period being held tightly laterally by any mechanical means and se- 100 cured by locking.

When making very light ingots, of which the solidification is almost instantaneous, the two operations may be combined into one, filling the ingot-mold with its smaller end at 105 the bottom when resting on the plane surface of a metallic block, lifting it immediately with the ingot in it, carrying it while holding it

vertically to a press similar to the press B in Fig. 1, where it is seized laterally, the smaller end being free and still directed downward, and, last, causing a mechanical or hydraulic ram to descend onto the larger end and advance the metal and force it out of the smaller end of the cone.

- In order to mechanically and rapidly force small ingots into and through conical molds,
- 10 I have devised the arrangement of ingot-mold shown in Fig. 2, which is more particularly adapted for use when the complete operation is condensed in one period. The ingot-mold *a*, which is made slightly conical both 15 inwardly and outwardly and strengthened by hoops *b*, is provided at the bottom with a collar *f*, by means of which it is centered on a lower portion or hollow block *d*, fixed to the foundation *e* of the press, which serves to 20 force the ingot out through the smaller end of the mold *a*. The orifice of the block *d* is cylindrical at the portion *g*, which forms a prolongation of the ingot-mold and is of the same diameter as its lower base. It is then made 25 highly conical at *h* and terminates in a cylindrical portion *i*. When it is desired to force the ingots *c* into and through the mold in a single operation, the conical ingot-mold *a* is first placed upon a flat metal bottom for the 30 purpose of casting. When it has received the steel which forms the ingot *c*, it is rapidly placed upon the block *d*, fixed to the foundation *e* of the press C, Fig. 3. The ingot-mold being thus arranged on the block *d*, the ram *t*, 35 actuated by the cylinder *p* of the press C, is lowered onto the upper face of the ingot *c*, which is still in a great measure fluid. The ram causes the metal to pass from the large end of the ingot-mold toward the small end 40 and toward the block in which the compression is carried out. In order to cool the ingot directly after compression and in order to prevent swelling, water or steam is brought into contact with the metal. The water or 45 steam passes under pressure into the block through the nozzle *j* and into the annular pipe *k*, from whence it passes through the pipe *l* into the central orifice.
- In place of causing the ram of the press to 50 act until the ingot passes completely out through the small end of the ingot-mold it may be stopped a little prior to this and the ingot thus compressed taken out through the top by pushing it mechanically from below 55 by any suitable means, such as a push-back ram *s*, Fig. 3, of a diameter smaller than that of the narrowest part of the block *d* or the mold *a*. It is above all of importance in this case to prevent swelling, which would render 60 the return of the ingot very difficult.

Having thus described the nature and ob-

jects of my invention, what I claim as new, and desire to secure by Letters Patent, is—

1. In an apparatus of the character described, a vertical ingot-mold having a slightly 65 conical cavity, means forming the continuation for the smaller end of said mold at the base and wherein an ingot is adapted to be solidified by compression when forced out through said mold and the means forming the 70 continuation of the smaller end of said mold.

2. In an apparatus of the character described, a slightly frusto-conical ingot-mold, a hollow block arranged adjacent to and forming the continuation for the smaller end of 75 said ingot-mold, and the hollow portion of said block having successive cylindrical frusto-conical and cylindrical portions.

3. In an apparatus of the character described, a vertical ingot-mold having a slightly 80 conical cavity, the smaller diameter of which is at the base of the mold, a hollow block for centering and supporting the mold at its base having a highly conical portion located between two cylindrical portions, forming the 85 continuation of the cavity of the mold to still further compress and to solidify the ingot when forced out of the cavity of the mold into and through said hollow block.

4. In an apparatus of the character described, a slightly frusto-conical ingot-mold, a hollow block arranged adjacent to and forming the continuation for the smaller end of 90 said ingot-mold, the hollow portion of said block having successive cylindrical frusto-conical and cylindrical portions, to further 95 compress the ingot forced through the successive portions of said block, in combination with means for circulating a cooling medium in said block during passage of the ingot therethrough.

5. In an apparatus of the character described, a slightly frusto-conical ingot-mold for solidifying an ingot by compression, a hollow block arranged adjacent to and forming 105 the continuation for the smaller end of said ingot-mold, the hollow portion of said block having successive frusto-conical and cylindrical portions to further compress the ingot when forced into and through said block, in combination with means for circulating a cooling medium in said block during the passage of the ingot therethrough, and pushing 110 of the ingot back through said block.

In testimony whereof I have signed this 115 specification in the presence of two subscribing witnesses.

HENRI HARMET.

Witnesses:

HASTINGS BURROUGHS,  
J. BEARLET.